

## UNITED STATES PATENT OFFICE

1,998,389

## PROCESS FOR IMPROVING CELLULOSE

Emil Scheller, Lorsbach in Taunus, Germany

No Drawing. Application November 12, 1930.  
Serial No. 495,301. In Germany November 23,  
1929

4 Claims. (CL. 8—2)

In my previous patent application S. N. 477,191 I have applied for a process for improving celluloses, which allows of obtaining products having particular properties, such as for instance a high degree of bleach, high or adjustable content of undecomposed alpha-cellulose, small content of ash, and low copper number.

The process of my invention Serial No. 477,191 consists essentially in this that the cellulose to be treated is subjected successively to a treatment with chlorine, an alkaline treatment at increased temperature, preferably with exclusion of elementary oxygen and a treatment with active oxygen or with or without unrestricted admission of air, whereupon the process is terminated by acidifying the material. By elemental oxygen is meant oxygen in the gaseous state. By active oxygen is meant oxygen existing in combined form in oxidizing agents, such as metal peroxides, hydrogen peroxide and other well known oxidizing agents. This combined oxygen is readily released from the oxidizing agent during the course of the process, and is available for use in the process. Active oxygen is sometimes known as nascent oxygen.

According to the process of my earlier application, Serial No. 477,191, the cellulose is subjected to a treatment which is, in brief, as follows:

The cellulose material is first bleached in the usual manner by the use of a chlorine bleach. The quantity of chlorine here employed can advantageously be less than that which is usual in the art. This results in obtaining an article which is bleached from  $\frac{1}{2}$  to  $\frac{3}{4}$  white.

The material is then thoroughly washed, and afterward is subjected to a treatment with an alkaline solution at ordinary or increased pressures and at high temperatures. Air should be excluded during this treatment, for example, the process may be carried out in an autoclave. In general, the highest content of alpha cellulose is obtained by the use of sodium hydroxide. One can, however, use sodium carbonate, lime, or a mixture of the two. The quantity of alkali employed will depend upon the quality of the cellulose and is preferably so limited that immediately after the boiling process the liquor still gives an alkaline reaction. Ordinarily, 5 to 10% of caustic alkali, based on the dry weight of the cellulose will prove satisfactory. Boiling for longer periods and at increased pressure increases the quantity of alpha cellulose. In case the pre-treatment with chlorine has been longer than is recommended, i. e. if the goods are bleached more than  $\frac{1}{2}$  to  $\frac{3}{4}$

white it is necessary to carry out a more energetic alkali treatment in order to produce a high content of alpha cellulose. The working conditions should, therefore, be naturally arranged to obtain the most suitable action according to the nature of the cellulose employed.

Following the caustic alkali boil, the material is washed out thoroughly and then subjected to the oxygen bleach. It has been found that the quality of the product obtained, and more particularly the viscosity of solutions of this product which are made, for example, by dissolving the product after treatment in carbon bisulphide plus sodium hydroxide or in ammoniacal copper solutions, may be varied to a considerable extent by regulating the amount of molecular or elemental oxygen present during the bleaching process, as by excluding elemental oxygen entirely or admitting varying quantities thereof. This regulation of the oxygen present is especially important during the bleaching with the alkali metal peroxides. If the elementary oxygen is entirely absent during this treating stage, a product giving solutions of very high viscosity is produced, on the other hand, to obtain solutions of varying viscosity, as is sometimes desired, measured amounts of oxygen may be intentionally introduced.

Alkaline solutions of hydrogen peroxide, obtained from sodium peroxide, are the most advantageous sources of active oxygen. The amount of sodium peroxide employed will in general range from 1 to 2% of the weight of the goods.

This is a summary of the process disclosed in my earlier application. I have now made further investigations and have improved this earlier process. These subsequent experiments have shown that it is advantageous to precede the treatment of the material with chlorine, by an alkaline treatment at increased temperature which in this case also is carried out with or without the exclusion of elementary oxygen. This preliminary treatment may consist in boiling the material at ordinary or increased pressure in alkaline lye, preferably a caustic alkali lye.

The subsequent treatment with chlorine is preferably in the form of a partial bleach, for instance in such a way that the quantities of chlorine acting upon the material are so restricted that for instance the bleach is only  $\frac{1}{2}$  to  $\frac{3}{4}$  white.

I have also found that with this method of treatment, an intermediate alkaline boiling, such as takes place according to the said previous patent application Serial No. 477,191 between the chlorine treatment and the treatment of the ma-

terial with active oxygen, can if desired be dispensed with.

The present process enables the carrying out of the process with a smaller expenditure of bleaching media, products being obtained, which are equal to those of the said previous patent application or in some cases even have better properties. In other respects the working conditions of the previous patent application apply for carrying out the present process. This applies more especially as regards the exclusion or admission of oxygen from the air. For instance according to the desired viscosity properties of the finished cellulose, elementary oxygen may either be completely excluded or restricted or even unrestricted access given thereto.

According to the nature of the initial material and the particular requirements to be satisfied by the end product, one boiling in alkali may be sufficient or, if necessary, in addition to the alkaline preliminary treatment preceding the chlorination, a further boiling in alkali will be interposed between the treatment with chlorine and the oxygen bleach.

After bleaching, the goods are washed and acidified. This acidification is preferably carried to a point where the solution is weakly acid, as indicated by the Congo red acid reaction. This has a favorable effect in decreasing the ash content, provided the goods are subjected to a careful and thorough washing out afterwards. The latter part of this washing out is generally conducted in the presence of small quantities of alkali or ammonia.

It will be understood that the matter of regulating the time of bleaching, the temperature and the alkalinity will vary considerably according to the quality of the material with which one starts, and also according to the qualities which one desires to impart to the final product, and I, therefore, do not desire to be limited to the specific disclosures of this kind which have been given here largely by way of example. It must be understood that in art of this kind one necessarily must determine experimentally certain features of the process which are inherently subject to variation.

By following the method herein described, I have obtained as an example a cellulose with a content of 96.26% alpha-cellulose.

The improvement obtainable by the present

process is clear from the following comparative example:

|                                            | Results obtained by process of the previous application S. N. 477,191 | Results obtained by the process of this application |
|--------------------------------------------|-----------------------------------------------------------------------|-----------------------------------------------------|
| Cellulose                                  | Percent 94.26                                                         | Percent 95.54                                       |
| Consumption of chlorine                    | 0.9                                                                   | 0.55                                                |
| Na <sub>2</sub> O <sub>2</sub> consumption | 1.25                                                                  | 0.5                                                 |

What I claim is:

1. A process for improving cellulose which comprises treating such cellulose with alkali at increased temperatures, thereupon partially bleaching the same with chlorine, subsequently completing the bleaching with an active oxygen containing substance capable of yielding hydrogen peroxide under the conditions of the process and then acidifying the material.

2. A process for improving cellulose which comprises treating such cellulose with alkali at increased temperatures in the presence of definite quantities of oxygen, thereupon partially bleaching the same with chlorine, subsequently completing the bleaching with an active oxygen containing substance capable of yielding hydrogen peroxide under the conditions of the process and then acidifying the material.

3. A process for improving cellulose which comprises treating such cellulose with alkali at increased temperatures, thereupon partially bleaching said cellulose with chlorine, then treating said cellulose again with alkali at increased temperatures, subsequently completing the bleaching with an active oxygen containing material capable of yielding hydrogen peroxide under the conditions of the process, and then acidifying said material.

4. A process for improving cellulose which comprises treating said cellulose with alkali at increased temperatures, thereupon partially bleaching the same with chlorine, and subsequently completing the bleaching with an active oxygen containing substance capable of yielding hydrogen peroxide under the conditions of the process while regulating the quantity of elemental oxygen present, and then acidifying the material.

EMIL SCHELLER.